

## UNITED STATES PATENT OFFICE

2,159,011

PRODUCTION OF YARNS, FABRICS, ETC.,  
HAVING A BASIS OF ORGANIC DERIVA-  
TIVES OF CELLULOSE

Henry Dreyfus, London, England

No Drawing. Application September 5, 1935, Se-  
rial No. 39,289. In Great Britain September 11,  
1934

3 Claims. (Cl. 8—121)

This invention relates to improvements in the production of yarns, fabrics and other materials, and is more particularly concerned with processes for the production of cellulose derivative yarns, fabrics and other materials, and with the new yarns, fabrics and other materials produced thereby.

I have found that the resistance to heat of cellulose acetate yarns, fabrics and other materials may be increased by subjecting yarns and other materials to esterification with acid anhydrides, for example by treatment with diluted acetic anhydride, in the presence of metallic halide catalysts. By this means the melting point and the safe ironing point of yarns and similar materials may be increased so that they may be ironed without damage at higher temperatures than are customary in ironing ordinary cellulose acetate artificial silk. In addition, the treatment reduces the moisture regain of the materials and they acquire a greater resistance to water, and have a substantially greater resistance to the delustring action of hot or boiling aqueous liquids or moist steam. In addition, the affinity of the materials for dye-stuffs in general, and particularly for the dispersed insoluble dyestuffs now commonly applied to cellulose acetate, is materially reduced, so that by association of the yarns or other materials so treated with yarns or other materials of cellulose acetate or of other organic derivatives of cellulose untreated by the process, differential dyeing effects are obtainable, whilst at the same time the dye has an affinity for the whole of the fabric or other material in which the two types of yarn are associated. Thus, for instance, light and dark blue shades can be produced by the immersion in a dyebath containing an SRA blue dyestuff of a fabric containing ordinary acetone-soluble cellulose acetate yarn together with the same yarn which has been subjected to the process of the invention.

In a similar manner cellulose acetate artificial silk and other materials may be treated with other acid anhydrides to produce a similar effect and, in addition, artificial silks and other materials of other organic derivatives of cellulose may be subjected to treatment with acetic anhydride or other acid anhydride. Examples of other lower organic acid anhydrides which may be employed are propionic and butyric anhydrides.

In addition to increasing the resistance to heat and the resistance to water, the new process has the effect of changing the solubility characteristics of the yarns or similar materials. Thus, for instance, by treating cellulose acetate yarn with

acetic anhydride or other acid anhydride according to the present invention, a yarn may be produced which is insoluble or much less soluble in acetone. Similar changes in the solubility characteristics occur in the treatment of other yarns used as starting materials in the treatment of the invention. It is thus possible, according to the invention, to produce yarns which it is difficult or even impossible to manufacture by a simple spinning process.

According to the present invention, therefore, artificial yarns, fabrics and other materials having improved properties are obtained by acetylation or otherwise esterifying such materials having a basis of an organic derivative of cellulose by means of organic acid anhydrides in the presence of metal halide catalysts.

The invention will hereinafter be described particularly with reference to the esterification of the yarns, but it is to be understood that it is also applicable to fabrics and other materials.

The acetic anhydride or other acid anhydride is diluted with a diluent which is a non-solvent for the yarn under treatment and which may be inert thereto, which is particularly useful where the anhydride has a strong swelling or dissolving action upon the yarn, or which may have a swelling action on the yarn. Good results are obtained with hydrocarbon diluents, for example xylene or other homologues of benzene, tetra- and decahydronaphthalenes, and kerosene or other high boiling petroleum hydrocarbons and also ethers, e. g., normal and isobutyl and amyl ethers, carbon tetrachloride and other non-solvent chlorinated hydrocarbons.

The degree of dilution may be adjusted so as to prevent swelling or so as to obtain some swelling of the yarn. In any case, it should be such as to prevent any solution or incipient solution of the yarn or any fusing together of the filaments, and, further, it may be adjusted to prevent any substantial change in the lustre or quality of the material. A given amount of acetic anhydride may, for example, be dissolved in 7 or 8 or 10 up to 20 times or more its weight of xylene or other hydrocarbon. The higher dilutions are particularly conducive to avoiding change in the lustre and in quality. The amount of acetic anhydride on the weight of the yarn may vary very considerably, but it is usually sufficient to use an amount of anhydride from half to twice the weight of the material, for example a proportion of 1-1½ times its weight. The proportion may be varied according to the degree of acetylation required and the amount of the change in the properties of

the material which it is desired to bring about. The same considerations apply with other acid anhydrides.

The reaction may be carried out under atmospheric pressure, sub-atmospheric pressure, or at pressures in excess of atmospheric, for example pressures of 20 pounds per square inch or more.

Esterification according to the present invention is, as stated above, carried out in the presence of metal halide catalysts. The catalysts which are particularly valuable for the process of the present invention are the halides of zinc and tin, for example zinc chloride and stannic chloride. Other catalysts which may be employed either separately or together are the halides, and particularly the chlorides, of chromium, iron, cobalt, antimony, bismuth, copper and mercury, for example antimony tri- and penta-chlorides, ferric bromide and iodide and cupric chloride and bromide. Preferably a hydro-halide acid is also present in suitable proportions which will depend to some extent upon the particular acid employed. For example, when acetylation cellulose acetate materials with acetic anhydride using zinc chloride as a catalyst, suitable proportions of hydrochloric acid are of the order of 1-5 or 10 molecular proportions of acid to 1 molecular proportion of zinc chloride. If hydrobromic or hydriodic acid is employed, in general somewhat higher proportions are desirable than with hydrochloric acid under similar conditions. It appears that the presence of the hydrohalide acid accelerates the reaction so that a given degree of esterification can be effected in a shorter time. Preferably the hydrohalide acid is introduced into the esterifying medium in the form of the dry gaseous hydrogen halide.

The catalyst may be present in the reaction mixture or may be present on the yarn before it is brought into contact with the reaction mixture. Where the yarn is previously impregnated with the metal halide catalyst, it is preferable to apply a solution of the desired catalyst and to dry the catalyst in the yarn before bringing the yarn into contact with the reaction medium.

The amount of catalyst employed will depend somewhat on the catalyst. However, the catalysts, for example, zinc chloride, stannic chloride or mixtures thereof with hydrochloric acid are preferably employed in quite low concentrations and are also preferably dissolved in the reactants.

Zinc chloride may, for example, be employed in a concentration in the reagents used for esterification of under 1%, for example .5%. The catalyst should not be employed in a sufficiently high concentration to bring about reaction between the anhydride employed and any diluent if such reaction is possible. For instance, with certain aromatic hydrocarbons acetic anhydride will react in the presence of zinc chloride and similar acidic catalysts if present in a sufficiently high concentration.

In general the lower the concentration of the esterifying agent or catalyst, the longer will the time of treatment be. It may, for example extend to 30 minutes or 1 hour up to 5 hours or more. The conditions necessitating these longer periods of treatment appear to be conducive to greater uniformity of reaction.

The most important starting material for the purpose of the present invention is the ordinary commercial acetone-soluble cellulose acetate yarn. Other suitable starting materials include

yarns of other esters of cellulose, for instance cellulose formate, propionate, butyrate and the like, and of ethers of cellulose, for instance methyl, ethyl and benzyl celluloses, and of ether-esters of cellulose, e. g., ethyl cellulose acetate.

For the purpose of brevity, the term "yarn" has been used, but it will be understood that the yarn may be treated in any suitable form, for example in the form of hanks, or on perforated bobbins or in the form of woven or warp-knitted or other knitted fabrics or similar materials.

The starting material may be a yarn produced by the ordinary spinning process, for example the well-known commercial acetone-soluble cellulose acetate yarn, or it may be a yarn treated by any suitable after-treatment process, for example stretching, shrinking, dyeing or other processes. For example, the yarn subsequent to its manufacture may be subjected to a stretching treatment designed to increase its tenacity, e. g. with the aid of a solution of dioxane or other suitable solvent, or in the presence of steam or hot water, as described in U. S. applications S. Nos. 4,510 filed February 1, 1935, and 4,511 filed February 1, 1935. The stretching treatment may, for example, be such as to extend the yarn by 200-500% or even 1000% or more of its original length. Such yarns have an extremely high tenacity which is reflected in the final product, treated according to the present invention. Such stretched yarns, or even ordinary artificial silk materials may, if desired, be subjected to a shrinking treatment to increase their extensibility, for example a shrinking treatment carried out with the aid of latent solvents (see U. S. application S. No. 611,240 filed May 13, 1932 now Patent No. 2,058,422, dated October 27, 1936).

The reaction between the cellulose derivative yarn and the acetic anhydride or other acid anhydride may be carried out in any suitable manner, for example as a batch process. For example hanks may be immersed for the appropriate period in the esterification mixture, or the mixture may be pumped or sucked through a perforated bobbin or other package of the yarn.

The following examples are given in order to illustrate the invention, but it is to be understood that they do not limit it in any way. The parts given are by weight in each case.

#### Example 1

70 parts of acetone-soluble cellulose acetate yarn are treated for about  $\frac{1}{4}$  of an hour at 20°-25° C. in a solution containing 200 parts of acetic anhydride, 800-900 parts of benzene, 10 parts of zinc chloride and 4 parts of hydrogen chloride. The yarn is then removed, washed first with benzene and then with water and dried.

#### Example 2

20 parts of yarn are treated for about 2 hours at 20°-25° C. in a mixture consisting of 400 parts of benzene, 40 parts of acetic anhydride, 2 parts of zinc chloride and 0.2 parts of hydrogen chloride. The yarn is then removed, washed with benzene and water and dried.

#### Example 3

20 parts of yarn are treated for about 2 hours at 20°-25° C. in a mixture consisting of 400 parts of benzene, 40 parts of acetic anhydride, 4 parts of zinc chloride and 1 part of hydrogen chloride. The yarn is then removed, washed with benzene and water and dried.

The yarn obtained according to each of the

preceding examples is chloroform-soluble, has an increased acetyl value, an improved resistance to ironing and to treatment with hot aqueous media and a decreased affinity for the ordinary cellulose acetate dyestuffs.

While the invention has been described above more particularly with reference to yarns, it may also be applied to films, foils and similar materials of cellulose derivatives. The expression 10 "non-solvent" liquid medium as used in the following claims is to be understood as meaning a medium which is a non-solvent for the materials being treated throughout the whole of the reaction.

15 What I claim and desire to secure by Letters Patent is:

1. Process for the production of improved artificial materials, which comprises subjecting 20 yarns, threads, fabrics and similar textile materials having a basis of acetone-soluble cellulose acetate to acetylation with a non-solvent liquid

medium comprising acetic anhydride, an organic diluent, stannic chloride and hydrochloric acid until they have a reduced solubility in acetone.

2. Process for the production of improved artificial materials, which comprises subjecting 5 yarns, threads, fabrics and similar textile materials having a basis of acetone-soluble cellulose acetate to acetylation with a non-solvent liquid medium comprising acetic anhydride, an organic diluent, zinc chloride and hydrochloric acid until 10 they have a reduced solubility in acetone.

3. Process for the production of improved artificial materials, which comprises subjecting 15 yarns, threads, fabrics and similar textile materials having a basis of acetone-soluble cellulose acetate to acetylation with a non-solvent liquid medium comprising acetic anhydride, an organic diluent, a metallic halide and a hydrohalide acid until they have a reduced solubility in acetone.

20

HENRY DREYFUS.